



US006020100A

# United States Patent [19]

Iwasaki et al.

[11] Patent Number: 6,020,100

[45] Date of Patent: Feb. 1, 2000

[54] **COLOR TONER MANUFACTURING METHOD, COLOR TONER MASTER BATCH, AND COLOR TONER**

[75] Inventors: **Yoshiaki Iwasaki**, Toyonaka; **Koshiro Nakao**, Nishinomiya; **Hiroshi Nakamura**, Kobe; **Shigeyuki Hakumoto**, Toyonaka, all of Japan

[73] Assignee: **Minolta Co., Ltd.**, Osaka, Japan

[21] Appl. No.: **09/045,376**

[22] Filed: **Mar. 20, 1998**

[30] **Foreign Application Priority Data**

Mar. 21, 1997 [JP] Japan ..... 9-067861  
Mar. 21, 1997 [JP] Japan ..... 9-067862  
Mar. 21, 1997 [JP] Japan ..... 9-067863  
Mar. 21, 1997 [JP] Japan ..... 9-067864

[51] **Int. Cl. 7** ..... **G03G 9/08**

[52] **U.S. Cl.** ..... **430/106; 430/137**

[58] **Field of Search** ..... 430/106, 109,  
430/137

[56]

## References Cited

### U.S. PATENT DOCUMENTS

5,272,034 12/1993 Kawano et al. .... 430/137  
5,300,383 4/1994 Tsubota et al. .... 430/45  
5,863,692 1/1999 Nakamura et al. .... 430/137

### FOREIGN PATENT DOCUMENTS

62-030259 9/1987 Japan .

*Primary Examiner*—John Goodrow

*Attorney, Agent, or Firm*—McDermott, Will & Emery

[57]

## ABSTRACT

A method of producing a color toner whereby a binder resin, a chromatic coloring material and a metal oxide particulate material are mixed to obtain a first mixture. Thereafter, a second mixture is obtained by mixing the first mixture with a material other than the materials used to obtain the first mixture. The second mixture is melted, kneaded, cooled and pulverized.

**25 Claims, 1 Drawing Sheet**

Fig. 1



**COLOR TONER MANUFACTURING  
METHOD, COLOR TONER MASTER BATCH,  
AND COLOR TONER**

**RELATED APPLICATIONS**

The present invention is based on Japanese Patent Application Nos. 9-67,861, 9-67,862, 9-67,863 and 9-67,864, each content of which is incorporated herein by reference.

**FIELD OF THE INVENTION**

The present invention relates to a method of manufacturing color toners for use in full color image forming apparatuses, such as full color electrostatic copying machine and full color laser beam printer, color toner master batch, and color toner.

**BACKGROUND OF THE INVENTION**

In a conventional image forming method which has been widely employed in copying machines, printers, facsimile, and the like, an electrostatic latent image formed on an electrostatic latent image supporting member, such as a photosensitive member, is developed by a toner, and the resulting toner image is transferred onto a recording member, such as recording paper, for image formation. In recent years, a full-color image forming apparatus for reproducing a multicolor image by superposing plural colors one over another has been put in practical application.

In such a full-color image forming apparatus, an electrostatic image is formed in dot units on an organic photosensitive member which is negatively charged by digital writing, for example, light beam irradiation, and the latent image is developed in reverse by using negatively chargeable magenta, cyan, and yellow toners, and black toner as required. Toner images of different colors thus obtained are superposed one over another so as to be reproduced as a multicolor image.

Such full-color image formation is largely utilized in reproducing pictures, photographs, graphic images and, as mentioned above, color toners of plural colors are superposed one over another for multicolor image reproduction. Such multicolor imaging is widely employed not only for image formation on recording paper, but also for image formation on overhead projector transparent sheets (OHP sheet). However, even though the color toner has distinct color reproducibility when a color toner image is formed on the recording paper, there is a problem that if such an image, formed on an OHP sheet, is actually projected onto a screen, the image becomes somewhat blackish, thus showing reduced color reproducibility.

**SUMMARY OF THE INVENTION**

It is an object of the present invention to provide a method of producing a color toner having good color developing characteristics and transparency when image formation is made on any recording paper or on any OHP sheet.

It is another object of the invention to provide a color toner master batch having good color developing characteristics and transparency when image formation is made on any recording paper or on any OHP sheet.

It is another object of the invention to provide a color toner having good color developing characteristics and transparency when image formation is made on any recording paper or on any OHP sheet.

The present invention relates to a method of producing a color toner which comprises the following steps:

a first mixing step for mixing a binder resin, a chromatic coloring material, and metal oxide particulate, wherein the weight ratio of the chromatic coloring material to the metal oxide particulate is 10:1-1:5;

a second mixing step for mixing the mixture obtained at the first mixing step and a material other than the materials used in the first mixing step;

the step of melting and kneading the mixture obtained at the second mixing step;

the step of pulverizing the kneaded mixture after the mixture has been cooled; and the step of classifying the resulting pulverized material.

The present invention further relates to a method of producing a color toner which comprises the following steps:

a first mixing step for mixing a binder resin having a mean particle size of 1 to 3 mm, and a chromatic coloring material;

a second mixing step for mixing the mixture obtained at the first mixing step and a binder resin having a mean particle size of 0.1 to 0.5 mm;

the step of melting and kneading the mixture obtained at the second mixing step;

the step of pulverizing the kneaded mixture after the mixture is cooled; and

the step of classifying the resulting pulverized material. The present invention further relates to a master batch for use in a color toner comprising:

a binder resin, 20 to 100 parts by weight of a chromatic coloring material relative to 100 parts by weight of the binder resin, and metal oxide particulate.

The present invention further relates to a method of producing a color toner which comprises the following steps:

a master batch preparing step for preparing a master batch containing a binder resin, 20 to 100 parts by weight of a chromatic coloring agent relative to 100 parts by weight of the binder resin, and metal oxide particulate;

a first mixing step for mixing the master batch and a binder resin;

a second mixing step for mixing the mixture obtained at the first mixing step and a material other than the materials used in the first mixing step;

the step of melting and kneading the mixture obtained; the step of pulverizing the kneaded mixture after the mixture is cooled; and

the step of classifying the resulting pulverized material.

The present invention further relates to a magenta toner comprising:

at least a binder resin and a magenta pigment; wherein when a film of the magenta toner is formed on a sheet for an overhead projector, the toner film has a surface gloss of 105 or more and satisfies the following relation (1):

$$(A_{MP} - A_{MB})/A_{MB} \geq 85 \quad (1)$$

in which  $A_{MP}$  denotes maximum absorbance of the toner film in a wave range of 500 to 600 nm, and  $A_{MB}$  denotes minimum absorbance in a wave range of 400 to 800 nm.

The present invention further relates to a yellow toner comprising:

at least a binder resin and a yellow pigment; wherein when a film of the yellow toner is formed on a sheet for an overhead projector, the toner film has a surface gloss of 105 or more and satisfies the following relation (2):

$$(A_{YP} - A_{YB})/A_{YB} \geq 75$$

(2)

in which  $A_{YP}$  denotes maximum absorbance of the toner film in a wave range of 380 to 500 nm, and  $A_{YB}$  denotes minimum absorbance in a wave range of 400 to 800 nm.

The present invention further relates to a cyan toner comprising:

at least a binder resin and a cyan pigment; wherein

when a film of the cyan toner is formed on a sheet for an overhead projector, the toner film has a surface gloss of 105 or more and satisfies the following relation (3):

$$(A_{CP} - A_{CB})/A_{CB} \geq 45$$

(3)

in which  $A_{CP}$  denotes maximum absorbance of the toner film in a wave range of 600 to 800 nm, and  $A_{CB}$  denotes minimum absorbance in a wave range of 400 to 800 nm.

#### BRIEF DESCRIPTION OF THE DRAWINGS

FIG. 1 is a view showing schematic construction of a full-color printer.

#### DESCRIPTION OF THE PREFERRED EMBODIMENTS

The method of producing a toner according to a first embodiment of the present invention is a mixing and pulverizing method for producing toner particles through steps of material-mixing, melting and kneading, pulverizing, and classifying. In the method, as will be explained hereinafter, the step of material mixing is carried out at plural stages, whereby dispersion characteristic of the chromatic coloring material can be improved, and this in turn results in improved color developing performance and improved transparency. The chromatic coloring material is usually obtainable in the form of fine primary particles during the process of synthesis thereof. However, when the coloring material is dried, secondary agglomeration occurs with the result that particles would become agglomerates having a volume mean particle size of 2 to 10  $\mu\text{m}$ . If a coloring material in the form of such secondary agglomerates is used, mere application of conventional mixing and grinding technique is not sufficient to cause the coloring material to be minutely dispersed into the toner, because the chromatic coloring material has high cohesive force. Therefore, the step of material mixing is divided into multiple stages to enable particular materials to be sequentially mixed so that dispersion of the coloring material in the form of secondary aggregation can be enhanced.

First, a binder resin, a chromatic coloring material, and metal oxide particles are mixed together at a first mixing step. At a second mixing step, a material other than the materials used in the first mixing step, such as a charge control agent and wax is introduced into and mixed with the mixture obtained at the first mixing step. In the case where dust size toner fine particles produced at pulverizing and classifying steps to be described hereinafter is to be collected and recycled as a material for toner production, such collected toner particles are introduced into and mixed with the mixture obtained at the second mixing step. At the first mixing step, coarse particles of binder resin having a volume mean particle size of 0.1 to 2 mm are used and a mixing operation is carried out by employing a mixing apparatus, such as Henschel mixer, which can exert shearing force upon the materials being mixed. By carrying out mixing in such a way, the secondary agglomerates of the coloring material are finely disintegrated into primary particles under a stress exerted when coarse particles of binder resin are mixed

while being ground. Further, the introduction of metal oxide fine particles results in the deposition of the metal oxide fine particles on the disintegrated coloring material, so that the chromatic coloring material which has been disintegrated into primary particles is prevented from becoming re-agglomerated. Further, because of the fact that such particulate material as charge control agent or collected dust-size toner particles is not introduced at the first mixing step, the shear force to be exerted on secondary agglomerates of the coloring material will not be lowered. Therefore, the secondary agglomerates can be effectively reduced to minute particle size. At the first mixing step, the chromatic coloring material and the metal oxide particulate are added in a weight ratio of chromatic coloring material to metal oxide particulate, of from 10:1 to 1:5, preferably 5:1 to 1:5. If the proportion of the metal oxide particulate is too small, no sufficient effect of such particulate could be obtained for the prevention of re-agglomeration of the chromatic coloring material and for improvement of the surface smoothness of toner-fixed film, and this results in degradation in color reproducibility and transparency. If the proportion of the metal oxide particulate is too large, the effect of glare prevention by the metal oxide particulate is excessively pronounced, so that the transparency of the toner is adversely affected.

For the metal oxide particulate it is desirable to use particles having a BET specific area of 20 to 300  $\text{m}^2/\text{g}$ , preferably 30 to 250  $\text{m}^2/\text{g}$ . As such metal oxide fine particles is it necessary to use colorless or white color particles, which will not affect the color reproducibility of the color toner, including for example silicon oxide (silica), titanium dioxide (titania), aluminum oxide (alumina), tin oxide, zinc oxide, and calcium oxide. From the viewpoint of environmental stability of the toner, for such metal oxide particulate, it is desirable to use hydrophobic particles which are surface-treated with a hydrophobicizing agent.

The chromatic coloring material and metal oxide fine particles only may be pre-mixed prior to the first mixing step. By carrying out such a pre-mixing step it is possible to efficiently cause metal oxide fine particles to deposit on the surface of the disintegrated chromatic coloring material to thereby prevent the re-agglomeration of chromatic coloring material particles during the process of toner preparation.

Next, as the second mixing step, a material other than the materials used in the first mixing step, such as a charge control agent and, where necessary, other material such as wax are introduced into and mixed with the mixture obtained at the first mixing step. In the case where collected dust-size toner particles are used as a material for toner preparation, such toner particles are introduced at the third mixing step, because the introduction of such particles at the second mixing step would lower the dispersibility of the charge control agent and the like.

By carrying out toner preparation in such a way it is possible to achieve minute dispersion of the coloring material without any such pretreatment as flush treatment of the chromatic coloring material or master batch treatment, to thereby reduce the cost of toner preparation.

According to the first embodiment described above, a toner having a volume-mean particle size of 4 to 9  $\mu\text{m}$ , with the chromatic coloring material minutely dispersed therein, can be obtained through the steps of melting and kneading the mixture obtained in the above multiple stage mixing, pulverizing the kneaded mixture after the mixture having been cooled, and classifying the resulting pulverized particles. The toner thus obtained has improved dispersion of

the chromatic coloring material, high transparency and good color reproducibility.

The method of producing a toner according to a second embodiment of the present invention is a mixing and pulverizing method for producing toner particles through steps of material mixing, melting and kneading, pulverizing, and classifying. In the method, as will be explained hereinafter, the step of material mixing is carried out at plural stages, whereby dispersion characteristic of the chromatic coloring material can be improved, and this in turn results in improved color developing performance and improved transparency.

First, a binder resin having a mean particle size of 1 to 3 mm, and a chromatic coloring material only are mixed at a first mixing step. A mixing operation is carried out by employing a mixing apparatus, such as Henschel mixer, which can exert shearing force upon the materials being mixed. Where binder resin particles having such a large particle size are mixed with the coloring material, particles of the coloring material which have become secondarily agglomerated are promptly disintegrated since the large-size binder resin particles exert a large amount of energy upon impingement thereof against the coloring material. However, once particles of the coloring material have been disintegrated to a certain extent, the coloring material will not become smaller in particle size any further. Whilst, where resin particles of small particle size and the coloring material are mixed together, it takes time to disintegrate the coloring material which has been secondarily agglomerated, because the impinging energy which will act on the coloring material is rather small. In this case, however, the coloring material can be more minutely disintegrated than in the case where resin particles of large particle size are used. From this point of view, at a second mixing step, the mixture obtained at the first mixing step using larger-size resin particles is admixed with smaller size resin particles having a mean particle size of 0.1 to 0.5 mm. Through the provision of this second mixing step the coloring material can be more finely disintegrated. At the second mixing step, materials other than those mixed at the first mixing step, for example, charge control agent and wax, may be introduced along with small-size resin particles for being mixed together. Further, it may be so arranged that at the second mixing step, small-size resin particles only are introduced into and mixed with the mixture obtained at the first mixing step, and that at a third mixing step, other material is introduced into the resulting mixture for being mixed therewith. By so doing it is possible to enhance the dispersion of the coloring material so that the resulting toner has improved color reproducibility.

Where dust-size toner particles produced at the pulverizing and classifying steps are collected and recycled as material for toner production, the collected toner particles may be introduced into and mixed with the mixture obtained through the above described mixing steps.

By carrying out toner preparation in such a way it is possible to achieve minute dispersion of the coloring material without any such pretreatment as flush treatment of the chromatic coloring material or master batch treatment, to thereby reduce the cost of toner preparation.

According to the second embodiment described above, a toner having a volume-mean particle size of 4 to 9  $\mu\text{m}$ , with the chromatic coloring material minutely dispersed therein, can be obtained after the steps of melting and kneading a mixture obtained through multiple stage mixing, pulverizing the kneaded mixture after the mixture having been cooled,

and classifying the resulting pulverized particles. The toner thus obtained has improved dispersion of the chromatic coloring material, high transparency and good color reproducibility.

A color toner master batch according to a third embodiment of the invention contains a high-concentration chromatic coloring material, a binder resin, and metal oxide particulate. By blending metal oxide particulate in this way it is possible to enhance the dispersion of the chromatic coloring material and improve toner transparency. Conceivably, the reason for the improvement in the dispersion of the coloring material may be explained by the fact that metal oxide particles deposit on particles of the disintegrated chromatic coloring material, which in effect prevents re-agglomeration of the chromatic coloring material. The reason for the improvement in transparency may be that the metal oxide particles serve to smooth the surface of a toner image after fixation, with the result that the possibility of irregular reflection on an image surface is reduced, which in effect leads to improved transparency. For the metal oxide particulate, particles similar to those used in the first embodiment may be used.

According to the third embodiment of the invention, a master batch is obtained by first mixing the materials, then melting and kneading the mixture, and pulverizing the kneaded mixture after having been cooled. More specifically, first, the chromatic coloring material, binder resin, and metal oxide fine particles are mixed together by a mixing apparatus, such as Henschel mixer, which can exert shearing force upon the materials being mixed. At this mixing step, disintegration of secondary agglomerates of chromatic coloring material occurs under a stress due to the shearing force of the mixer. In this conjunction, it may be arranged that prior to the mixing step, the chromatic coloring material and the metal oxide particulate are mixed and disintegrated and thereafter the mixture and the binder resin are mixed together, by so doing it is possible to further enhance the dispersion of the chromatic coloring material.

Then, the mixture is melted and kneaded, and the kneaded mixture is pulverized after having been cooled. The master batch is thus obtained. At this melting and kneading step, the coloring material is subjected to a large shearing force due to the high concentration of chromatic coloring material in the kneaded mixture, so that the coloring material is minutely dispersed.

The chromatic coloring material content of the master batch is 20 to 100 parts by weight, preferably 30 to 50 parts by weight, relative to 100 parts by weight of the binder resin. The weight ratio of the chromatic coloring material to the metal oxide particulate (coloring material: metal oxide) in the master batch is from 10:1 to 1:5, preferably from 5:1 to 1:5.

Then, the binder resin and, where necessary, additives, such as charge control agent and wax, are introduced into the master batch for being mixed therewith. The amount of addition of the binder resin to the master batch is so arranged that the coloring material content of the color toner finally obtained is 1 to 10 parts by weight relative to 100 parts by weight of the binder resin. A color toner having a volume-mean particle size of 4 to 9  $\mu\text{m}$ , with the chromatic coloring material minutely dispersed therein, can be obtained after the steps of melting and kneading the mixture obtained, pulverizing the kneaded mixture after the mixture having been cooled, and classifying the resulting pulverized particles. The color toner thus obtained has improved dispersion of the chromatic coloring material, high transparency and good color reproducibility.

In conjunction with the present invention, it has been found that the color reproducibility of color toner on an OHP sheet is dependent on the surface gloss of a toner film formed on the OHP sheet and, in turn, on the relation between maximum absorbance in a complementary wave range of the toner film and minimum absorbance (background absorbance) in a visible light range (400 to 800 nm). The degree of such dependence varies from color to color among different color toners and, therefore, color toners are prepared with adjustment within a specified range for each respective color toner, whereby good color reproduction on the OHP sheet can be achieved.

More specifically, in a magenta toner containing at least a binder resin and a magenta pigment, when a film of the magenta toner is formed on a sheet for an overhead projector, the toner film has a surface gloss of 105 or more and satisfies the following relation (1):

$$(A_{MP} - A_{MB})/A_{MB} \geq 85 \quad (1)$$

in which  $A_{MP}$  denotes maximum absorbance of the toner film in a wave range of 500 to 600 nm, and  $A_{MB}$  denotes minimum absorbance in a wave range of 400 to 800 nm.

In a yellow toner containing at least a binder resin and a yellow pigment, when a film of the yellow toner is formed on a sheet for an overhead projector, the toner film has a surface gloss of 105 or more and satisfies the following relation (2):

$$(A_{YP} - A_{YB})/A_{YB} \geq 75 \quad (2)$$

in which  $A_{YP}$  denotes maximum absorbance of the toner film in a wave range of 380 to 500 nm, and  $A_{YB}$  denotes minimum absorbance in a wave range of 400 to 800 nm.

In a cyan toner containing at least a binder resin and a cyan pigment, when a film of the cyan toner is formed on a sheet for an overhead projector, the toner film has a surface gloss of 105 or more and satisfies the following relation (3):

$$(A_{CP} - A_{CB})/A_{CB} \geq 45 \quad (3)$$

in which  $A_{CP}$  denotes maximum absorbance of the toner film in a wave range of 600 to 800 nm, and  $A_{CB}$  denotes minimum absorbance in a wave range of 400 to 800 nm.

The magenta toner to be used in the invention is such that the surface gloss of a magenta toner film formed on an OHP sheet is 105 or more. If the surface gloss is less than 105, transmitted light is reduced under the effect of irregular reflection on the surface of the toner layer, with the result that image transparency is reduced. While there is no particular upper limit of surface gloss, it is desirable that the surface gloss is less than 200, preferably about 150. Above noted values for the surface gloss are values measured according to the following method. First, an organic solvent solution with a toner dissolved therein was coated on an OHP sheet by a bar coat method so as to give a predetermined film thickness after dried. The glossiness of the toner film thus obtained was measured by using a gloss meter (GM-060; made by Minolta K. K.). The glossiness was calculated from the relation: (reflected luminous flux from sample/reflected luminous flux from standard glass) × 100. Measurement was made under the following conditions: angle of incidence and reflection of measured light was fixed at 60°; and glossiness of the standard glass having a refractive index of 1.567 was taken as 100. A magenta toner having above mentioned surface glossiness has good leveling characteristic such that its surface becomes smooth when the toner, melted at the stage of heat fixation, gets solidified.

In the magenta toner of the invention, the value of  $(A_{MP} - A_{MB})/A_{MB}$  in the above noted relation (1) is 85 or more, preferably 90 or more, more preferably 100 or more. If the value is less than 85, the transparency and color developing characteristic of the magenta toner on the OHP sheet will be lowered. There is no particular need for setting an upper limit for the value, though theoretically it is desirable that the value is larger. However, in view of the fact that above mentioned characteristic would become visually saturated and from the view point of the cost required for enhancement of dispersion, it is desirable that the value be not more than 500, preferably not more than 300. It is to be noted that the value has a correlation with the dispersion of the coloring material in the toner such that the value tends to become larger as dispersed particles of the coloring material are reduced in size. Aforesaid absorbance values are based on measurements made by using a self-recording spectro-photometer (U-3200; made by Hitachi Seisakusho K. K.) with respect to spectroscopic absorbance of toner films formed on the OHP sheet in a wave range of 400 to 800 nm.

In the present invention, the yellow toner to be used is such that the surface gloss of a yellow toner film formed on an OHP sheet is 105 or more. If the surface gloss is less than 105, transmitted light is reduced under the effect of irregular reflection on the surface of the toner layer, with the result that image transparency is reduced.

In the yellow toner of the invention, the value of  $(A_{YP} - A_{YB})/A_{YB}$  in the above noted relation (2) is 75 or more, preferably 80 or more, more preferably 85 or more. If the value is less than 75, the transparency and color developing characteristic of the yellow toner on the OHP sheet will be lowered. There is no particular need for setting an upper limit for the value, though theoretically it is desirable that the value is larger. However, in view of the fact that above mentioned characteristic would become visually saturated and from the view point of the cost required for enhancement of dispersion, it is desirable that the value be not more than 500, preferably not more than 300.

In the present invention, the cyan toner to be used is such that the surface gloss of a cyan toner film formed on an OHP sheet is 105 or more. If the surface gloss is less than 105, transmitted light is reduced under the effect of irregular reflection on the surface of the toner layer, with the result that image transparency is reduced.

In the cyan toner of the invention, the value of  $(A_{CP} - A_{CB})/A_{CB}$  in the above noted relation (3) is 45 or more, preferably 50 or more, more preferably 55 or more. If the value is less than 45, the transparency and color developing characteristic of the cyan toner on the OHP sheet will be lowered. There is no particular need for setting an upper limit for the value, though theoretically it is desirable that the value is larger. However, in view of the fact that above mentioned characteristic would become visually saturated and from the view point of the cost required for enhancement of dispersion, it is desirable that the value be not more than 500, preferably not more than 300.

For the chromatic coloring material in the invention, various known dyes and pigments may be used including, but not limited to, magenta colorants, such as C. I. pigment red 1-19, 21-23, 30-32, 37-41, 48-55, 57, 63, 64, 68, 81, 83, 87-90, 112, 114, 122, 123, 163, 184, 202, 206, 207 and 209; yellow colorants, such as C. I. pigment yellow 1-7, 10-17, 23, 65, 73, 83 and 180, C. I. bat yellow 1, 3 and 20; and cyan colorants, such as C. I. pigment blue 2, 3, and 15-17. The chromatic coloring material content of the toner is 1 to 15 parts by weight, preferably 1 to 10 parts by weight, relative to 100 parts by weight of the binder resin.

For the binder resin in the color toner of the present invention, it is desirable to use a resin having particular melting characteristics so as to enable the toner, as a full color toner, to have good light transmission property and good color reproducibility. It is desirable that the binder resin should have a melting viscosity  $V_2$  at 100°C. of  $5 \times 10^4$  to  $1 \times 10^6$  poise, and that the ratio of melting viscosity  $V_1$  of the binder resin at 90°C. to the melting viscosity  $V_2$  ( $V_1/V_2$ ) should be 8 or more, preferably from 8 to 40. If  $V_1/V_2$  is less than 8, the surface smoothness of the image is unfavorably affected with the result that the image surface tends to cause irregular reflection. Further, from the standpoint of fixation, it is desirable to use a binder resin having a softening point of 90 to 115°C. As long as the binder resin has such characteristics, the resin can be used in the present invention irrespective of the kind of the resin. Examples of such resins include styrene-acrylic copolymer resins, polyester resins, and epoxy resins, which may be used in one kind alone or in combination of two or more kinds. Of these resins, polyester resins are particularly preferred.

In the present invention, a preferred polyester resin is a polycondensation product comprising an alcoholic component, mainly bisphenol A alkylene oxide adduct, and an acid component including a phthalo-dicarboxylic acid or a combination of a phthalo-dicarboxylic acid and a fatty dicarboxylic acid.

For the charge control agent, it is necessary to use a colorless, white or light-colored agent serving as such. Examples of such agent include chrome salicylate complex salt E-81, 82 (made by Orient Kagaku Kogyo K. K.), zinc salicylate complex salt E-84 (made by Orient Kagaku Kogyo K. K.), aluminum salicylate complex salt E-86 (made by Orient Kagaku Kogyo K. K.), calix arene compound E-89 (made by Orient Kagaku Kogyo K. K.), and boron benzylate complex salt.

Where necessary, waxes such as low molecular weight polypropylene wax, low molecular weight polyethylene wax, carnauba wax, and SASOL wax may be added for anti-offset property improvement and, in the case of non-magnetic one-component toner, for preventing toner deposition on the regulator blade and/or developing roller of the developing apparatus.

In the present invention, 0.2 to 3% by weight of inorganic fine particles may be externally added to the toner particles obtained through above described steps for adjustment of fluidity and/or chargeability of the toner. Examples of such inorganic fine particles are silica, titania, alumina, strontium titanate, and tin oxide, which may be used in one kind alone or in a mixture of two or more kinds. From the viewpoint of environmental stability improvement it is desirable to use inorganic fine particles which have been surface treated with a hydrophobicizing agent. Besides such inorganic oxide particles, fine resin particles having a particle size of not more than 1  $\mu\text{m}$  may be externally added for cleanability improvement.

The color toner of the present invention can be used as a two-component developer non-magnetic toner which is to be used in mixture with a carrier, or as a non-magnetic one component toner which is not to be used with a carrier.

## EXAMPLES

The invention will now be described in further detail with respect to several examples given below. It is to be understood, however, that the invention is in no way limited by these examples. The binder resin used in the following examples and comparative examples is a polyester resin A obtained from bisphenol A propylene oxide adduct/

bisphenol A ethylene oxide adduct/terephthalic acid. The polyester resin A has a softening point of 98°C. and a glass transition point of 62°C. The melting viscosity at 100°C. of the binder resin is  $1 \times 10^5$  poise, and the ratio of the melting viscosity at 90°C. to the melting viscosity at 100°C. is 9. In Examples 1 to 7 and Comparative Examples 1 to 6, a polyester resin A in the form of particles pulverized to a volume-mean particle size of about 0.8 mm was used as such.

For the softening point and melting viscosity, measurement was made with respect to 1.0 g of sample by using a flow tester (CFT-500; made by Shimadzu Seisakusho K. K.) and a die of 1.0 mm  $\times$  1.0 mm under the conditions: temperature rise, 3.0°C./min.; preheat time, 180 sec.; load applied, 30 kg; measurement temperature range, 60 to 140°C. For the softening point, the temperature at which efflux of half of the sample occurred was taken as such. Measurement of the glass transition point was made with respect to 10 mg of sample weighed using a differential scanning calorimeter (DSC-200; made by Seiko Denshi K. K.) and, with alumina used as a reference, a shoulder value of main endothermic peak within a temperature range of 30 to 80°C. was taken as the glass transition point.

### Example 1

First, 150 g of hydrophobic silica (TS500; made by Cabosil K. K. BET specific surface area,  $225 \text{ m}^2/\text{g}$ ), as metal oxide particulate, were introduced into a 9-liter capacity Henschel mixer (made by Mitsui Kozan K. K.), and disintegrated at a peripheral speed of 40 m/sec. for 90 sec. Then, 1 kg of the binder resin, 30 g of chromatic coloring material, C. I. pigment red 184, (secondary agglomerate volume mean particle size, about 2.5  $\mu\text{m}$ ), and 30 g of the disintegrated hydrophobic silica were introduced into the Henschel mixer and subjected to a first stage mixing at a peripheral speed of 40 m/sec. for 4 minutes. Into the resulting mixture were introduced a negative charge control agent (E-84; made by Orient Kagaku Kogyo K. K.), 5 g, and a carnauba wax (made by Kato Yoko K. K.), 20 g, and second stage mixing was carried out for 5 minutes at a peripheral speed of 40 m/sec. Into the mixture thus obtained were introduced 150 g of collected dust-size toner particles (classified fine toner particles of the same composition as the mixture), and third stage mixing was carried out at a peripheral speed of 40 m/sec. for 5 minutes.

The resulting mixture was kneaded in a twin-screw extruder-kneader (PCM-30; made by Ikegai Tekko K. K.) and, after having been cooled, the kneaded mixture was primarily crushed in a feather mill, and then the resulting coarse particles were pulverized in a jet mill. Fine particles thus obtained were minutely classified by means of an air classifier. As a result, magenta toner particles having a volume-mean particle size of 8.5  $\mu\text{m}$  were obtained. It is noted that volume-mean particle size measurement was made using a Coulter counter (made by Coulter Electronics K. K.).

Hydrophobic silica (TS500; made by Cabosil K. K.), 0.8 part by weight, was added to 100 parts by weight of toner particles thus obtained, and mixing was carried out for 2 minutes by using a Henschel mixer at a peripheral speed of 20 m/sec. Thus, magenta toner 1 was obtained.

A yellow toner 1 having a volume-mean particle size of 8.4  $\mu\text{m}$  was obtained in the same way as in the case of the magenta toner 1, except that C. I. pigment yellow 180 (secondary agglomerate volume-mean particle size, about 3  $\mu\text{m}$ ) was used as chromatic coloring material. Similarly, a

## 11

cyan toner 1 having a volume-mean particle size of 8.7  $\mu\text{m}$  was obtained in the same way as in the case of the magenta toner 1, except that C. I. pigment blue 15-3 (secondary agglomerate volume-mean particle size, about 2.5  $\mu\text{m}$ ) was used as chromatic coloring material.

## Example 2

Magenta toner 2, yellow toner 2, and cyan toner 2 were obtained in the same way as in Example 1, except that the addition of the hydrophobic silica was made in the amount of 10 g.

## Example 3

Magenta toner 3, yellow toner 3, and cyan toner 3 were obtained in the same way as in Example 1, except that the addition of hydrophobic silica was made in the amount of 3 g.

## Example 4

Magenta toner 4, yellow toner 4, and cyan toner 4 were obtained in the same way as in Example 1, except that for the hydrophobic silica, R972 (made by Aerosil Japan; BET specific surface area, 110  $\text{m}^2/\text{g}$ ) was used in the amount of 40 g.

## Example 5

Magenta toner 5, yellow toner 5, and cyan toner 5 were obtained in the same way as in Example 1, except that hydrophobic titanium dioxide (T805; made by Aerosil Japan; BET specific surface area, 35  $\text{m}^2/\text{g}$ ), 30 g, was used instead of hydrophobic silica.

## Example 6

Magenta toner 6, yellow toner 6, and cyan toner 6 were obtained in the same way as in Example 5, except that the addition of hydrophobic titanium dioxide was made in the amount of 120 g.

## Example 7

Magenta toner 7, yellow toner 7, and cyan toner 7 were obtained in the same way as in Example 1, except that prior to the first mixing step, 30 g of chromatic coloring material and 30 g of hydrophobic silica were premixed and disintegrated by using a surface modifier (hybridization; made by Nara Kikai Seisakusho K. K.), the first mixing step being carried out thereafter using the pre-mixed components and 1 kg of binder resin.

## Comparative Example 1

Magenta toner 8, yellow toner 8, and cyan toner 8 were obtained in the same way as in Example 1, except that all materials were mixed together for 15 minutes in one stage without being separated into parts.

## Comparative Example 2

Magenta toner 9, yellow toner 9, and cyan toner 9 were obtained in the same way as in Example 1, except that a binder resin and a chromatic coloring material only were mixed at the first mixing step, and that hydrophobic silica, carnauba wax, and a charge control agent were introduced into the first-stage mixture for mixing therewith at the second mixing step.

## Comparative Example 3

Magenta toner 10, yellow toner 10, and cyan toner 10 were obtained in the same way as in Example 1, except that

## 12

the amount of addition of hydrophobic silica at the first mixing step was changed to 1 g.

## Comparative Example 4

Magenta toner 11, yellow toner 11, and cyan toner 11 were obtained in the same way as in Example 1, except that no hydrophobic silica was added at the first mixing step.

## Comparative Example 5

Magenta toner 12, yellow toner 12, and cyan toner 12 were obtained in the same way as in Example 5, except that the quantity of addition of hydrophobic titanium dioxide was changed to 300 g.

## Comparative Example 6

Magenta toner 13, yellow toner 13, and cyan toner 13 were obtained in the same way as in Comparative Example 1, except that no hydrophobic titanium dioxide was added.

With respect to color toners (magenta toners, yellow toners, and cyan toners) 1-13 obtained in manner as described above, a full-color image was formed on an OHP sheet using a full-color printer of the non-magnetic one-component developing system which will be explained hereinafter. Each image thus formed was projected by OHP onto a screen, and the color image on the screen was visually evaluated. In color development evaluation, where good color reproduction was observed, the toner was rated  $\textcircled{O}$ ; where color reproduction was somewhat less favorable, the toner was rated  $\textcircled{O}$ ; where color reproduction was inferior, but color discrimination was possible, the toner was rated  $\Delta$ ; and where color discrimination was difficult, the toner was rated  $\text{x}$ . In transparency evaluation, where the image was found clear, the toner was rated  $\textcircled{O}$ ; where the image was found slightly less clear, the toner was rated  $\textcircled{O}$ ; where the image was found somewhat dark, the toner was rated  $\Delta$ ; and where the image was found dark, the toner was rated  $\text{x}$ . The results are shown in Table 1.

TABLE 1

|             | Color toner | Multi-stage mixing | Time for fine particle addition | Colorant:Fine particle | Color develop property                 | Transparency                           |
|-------------|-------------|--------------------|---------------------------------|------------------------|----------------------------------------|----------------------------------------|
| Ex. 1       | 1           | Yes                | First mixing                    | 1:1                    | $\textcircled{O} \sim \textcircled{O}$ | $\textcircled{O} \sim \textcircled{O}$ |
| Ex. 2       | 2           | Yes                | First mixing                    | 3:1                    | $\textcircled{O} \sim \textcircled{O}$ | $\textcircled{O}$                      |
| Ex. 3       | 3           | Yes                | First mixing                    | 10:1                   | $\textcircled{O}$                      | $\textcircled{O}$                      |
| Ex. 4       | 4           | Yes                | First mixing                    | 3:4                    | $\textcircled{O}$                      | $\textcircled{O} \sim \textcircled{O}$ |
| Ex. 5       | 5           | Yes                | First mixing                    | 1:1                    | $\textcircled{O} \sim \textcircled{O}$ | $\textcircled{O}$                      |
| Ex. 6       | 6           | Yes                | First mixing                    | 1:4                    | $\textcircled{O}$                      | $\textcircled{O}$                      |
| Ex. 7       | 7           | Yes                | First mixing                    | 1:1                    | $\textcircled{O}$                      | $\textcircled{O}$                      |
| Comp. Ex. 1 | 8           | No                 | Collective mixing               | 1:1                    | $\Delta$                               | $\textcircled{O}$                      |
| Comp. Ex. 2 | 9           | Yes                | Second mixing                   | 1:1                    | $\Delta$                               | $\textcircled{O}$                      |
| Comp. Ex. 3 | 10          | Yes                | First mixing                    | 30:1                   | $\Delta$                               | $\textcircled{X}$                      |
| Comp. Ex. 4 | 11          | Yes                | —                               | —                      | $\Delta$                               | $\textcircled{X}$                      |
| Comp.       | 12          | Yes                | First                           | 1:10                   | $\textcircled{O}$                      | $\Delta$                               |

TABLE 1-continued

| Color toner | Multi-stage mixing | Time for fine particle addition | Colorant:Fine particle | Color develop property | Transparency |
|-------------|--------------------|---------------------------------|------------------------|------------------------|--------------|
| Ex. 5       |                    | mixing                          |                        |                        |              |
| Comp.       | 13                 | No                              | —                      | x                      | x            |
| Ex. 6       |                    |                                 | —                      |                        |              |

The full-color printer employed for the purpose of this evaluation is of such a construction as shown in FIG. 1, and includes a photosensitive drum **10** (hereinafter referred to as "sensitive member **10**") driven to rotate in the direction of arrow in the drawing, a laser scan optical system **20**, a full-color developing assembly **30**, an endless intermediate transfer belt **40** driven to rotate in the direction of arrow in the drawing, and a sheet feeder portion **60**. Around the sensitive member **10** there are provided a charging brush **11** for charging the surface of the sensitive member **10** to a predetermined potential, and a cleaner **12** for removing any toner residue present on the sensitive member **10**.

The laser scan optical system **20** is a well-known system incorporating a laser diode, a polygon mirror, and an f0 optical element, and has a controller to which print data for cyan (C), magenta (M), yellow (Y), and black (BK) are transmitted from the host computer. The laser scan optical system **20** sequentially output print data for each respective color in the form of laser beam and scan over the sensitive member **10** for exposure, whereby electrostatic latent images for respective colors are sequentially formed on the sensitive member **10**.

The full-color developing assembly **30** is an integral assembly of four separate color developing units **31C**, **31M**, **31Y**, **31BK** in which are housed respective one-component developing agents composed respectively of non-magnetic C, M, Y and BK toners, and is rotatable clockwise about a support shaft **33**. Each color developing unit includes a developing sleeve **32**, toner regulator blades **34a** and **34b**. Toner particles transported through the rotation of the developing sleeve **32** are charged by their passing through a pressure contact portion (regulator portion) between the blades **34a**, **34b** and the developing sleeve **32**.

The intermediate transfer belt **40** is driven to rotate synchronously with the sensitive member **10** in the direction of the arrow shown in the drawing. The intermediate transfer belt **40** is pressed by a freely rotatable first transfer roller **41** into contact with the sensitive member **10**. The intermediate transfer belt **40** is in contact with a freely rotatable second transfer roller **43** at a portion supported by a support roller **42**.

A cleaner **50** is disposed in a space between the developing assembly **30** and the intermediate transfer belt **40**. The cleaner **50** has a blade for removing any toner residue on the intermediate transfer belt **40**. The blade and the second transfer roller **43** are movable toward and away from the intermediate transfer belt **40**.

The sheet feeder portion **60** includes a feed tray **61** adapted to open on the front side of the image forming apparatus **1**, a feed roller **62** and a timing roller **63**. Recording sheets **S**, loaded on the feeder tray **61**, are fed one by one rightward by the feed roller **62** and delivered by the timing roller **63** toward the second transfer section in synchronous relation with an image formed on the intermediate transfer belt **40**. A horizontal transport path for recording sheets comprises an air suction belt **66** and the like, including the

sheet feeder portion, and a vertical transport path **80** equipped with transport rollers extends from a fixing unit **70**. Each recording sheet **S** is discharged from the vertical transport path **80** onto the top surface of the image forming apparatus body **1**.

In this conjunction, printing operation of the full-color printer will be explained. When printing operation begins, the sensitive member **10** and the intermediate transfer belt **40** are driven to rotate at an equal peripheral speed, and the sensitive member **10** is charged by the charging brush **11** to a predetermined potential.

Subsequently, a cyan image is exposed by the laser scan optical system **20** so that an electrostatic latent image of the cyan image is formed on the sensitive member **10**. The electrostatic latent image is immediately developed at developing unit **31C** and a toner image is transferred onto the intermediate transfer belt **40** at the first transfer section. Immediately upon the completion of the first transfer, developing unit **31M** is switched over to the developing section **D**, followed by exposure, development and first transfer with respect to magenta image. Then, switching over to developing unit **Y** is carried out, followed by exposure, development, and first transfer with respect to yellow image. Again, switching over to developing unit **31BK** is carried out, followed by exposure, development, and first transfer with respect to black image. Each time when a first transfer is made, a toner image is placed on the intermediate transfer belt **40** in superposed relation to a previously placed toner image.

Upon completion of a final first transfer, recording sheet **S** is delivered to a second transfer section and a full-color toner image formed on the intermediate transfer belt **40** is transferred onto the recording sheet **S**. Upon completion of the second transfer, recording sheet **S** is transported to a belt-type heat fixing device **70**, and a full-color toner image is fixed on the recording sheet **S**, which is in turn discharged onto the upper surface of the printer body **1**.

#### Preparation of Binder Resin Particles A1 and A2

The polyester resin **A** was pulverized in a feather mill (screen: 3 mm), and resulting particles were sifted through a 28-mesh screen. Particles present on the screen were classified as binder resin particles **A1** (mean particle size: 1.8 mm), and particles which passed through the screen was classified as binder resin particles **A2** (mean particle size: 0.3 mm).

#### Preparation of Binder Resin Particles A3

The polyester resin was pulverized in a feather mill (screen: 5 mm), and resulting particles were sifted through an 8-mesh screen. Particles present on the screen were classified as binder resin particles **A3** (mean particle size: 3.7 mm).

#### Preparation of Binder Resin Particles A4

The binder resin particles **A2** were further sifted through a 120-mesh screen, and particles which have passed through the screen were classified as binder resin particles **A4** (mean particle size: 0.06 mm).

#### Example 8

Three hundred grams (300 g) of binder resin particles **A1**, and 30 g of chromatic coloring material, C. I. pigment red 184, (secondary agglomerate volume mean particle size, about 3  $\mu$ m) were introduced into a 9-liter capacity Henschel mixer and subjected to first-stage mixing wherein mixing was carried out at a peripheral speed of 40 m/sec. for 5 minutes. Into the resulting mixture were introduced binder resin particles **A2**, 700 g, and a negative charge control agent

## 15

(E-84; made by Orient Kagaku Kogyo K. K.), 10 g, and second stage mixing was carried out at a peripheral speed of 40 m/sec. for 4 minutes.

The resulting mixture was kneaded in a twin-screw extruder-kneader (PCM-30; made by Ikegai Tekko K. K.) and, after having been cooled, the kneaded mixture was primarily crushed in a feather mill, and then the resulting coarse particles were pulverized in a jet mill. Fine particles thus obtained were minutely classified by means of an air classifier. As a result, magenta toner particles having a volume-mean particle size of 8.6  $\mu\text{m}$  were obtained. It is to be noted that the volume-mean particle size values herein are based on measurements by a Coulter counter (made by Coulter Electronics).

10  
5  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8895  
8900  
8905  
8910  
8915  
8920  
8925  
8930  
8935  
8940  
8945  
8950  
8955  
8960  
8965  
8970  
8975  
8980  
8985  
8990  
8995  
9000  
9005  
9010  
9015  
9020  
9025  
9030  
9035  
9040  
9045  
9050  
9055  
9060  
9065  
9070  
9075  
9080  
9085  
9090  
9095  
9100  
9105  
9110  
9115  
9120  
9125  
9130  
9135  
9140  
9145  
9150  
9155  
9160  
9165  
9170  
9175  
9180  
9185  
9190  
9195  
9200  
9205  
9210  
9215  
9220  
9225  
9230  
9235  
9240  
9245  
9250  
9255  
9260  
9265  
9270  
9275  
9280  
9285  
9290  
9295  
9300  
9305  
9310  
9315  
9320  
9325  
9330  
9335  
9340  
9345  
9350  
9355  
9360  
9365  
9370  
9375  
9380  
9385<br

## 17

-continued

| Color toner | Time for large-size particle addition | Time for small-size particle addition | Color develop property | Transparency |    |
|-------------|---------------------------------------|---------------------------------------|------------------------|--------------|----|
| Ex. 7       | mixing                                |                                       |                        |              |    |
| Comp. 20    | —                                     | First                                 | x~Δ                    | x            |    |
| Ex. 8       |                                       | mixing                                |                        |              |    |
| Comp. 21    | First                                 | First                                 | Δ~○                    | x~Δ          | 5  |
| Ex. 9       | mixing                                | mixing                                |                        |              |    |
| Comp. 22    | First                                 | Second                                | x~Δ                    | x            | 10 |
| Ex. 10      | mixing                                | mixing                                |                        |              |    |
| Comp. 23    | First                                 | Second                                | Δ                      | Δ            |    |
| Ex. 11      | mixing                                | mixing                                |                        |              |    |
| Comp. 24    | First                                 | —                                     | Δ                      | ○            |    |
| Ex. 12      | mixing                                |                                       |                        |              |    |

In the following examples and comparative examples, polyester resin A pulverized to a volume-mean particle size of about 0.8 mm was used as binder resin.

## Master Batch Preparation Example 1

Five hundred and forty (540) g of above mentioned polyester resin, 230 g of chromatic coloring material, C. I. pigment red 184 (secondary agglomerate volume mean particle size, about 3  $\mu\text{m}$ ), and 230 g of hydrophobic silica (R972; made by Aerosil Japan; BET specific surface area, 110  $\text{m}^2/\text{g}$ ) were introduced into a 9-liter capacity Henschel mixer (made by Mitsui Kozan K. K.) and were mixed at a peripheral speed of 40 m/sec. for 4 minutes. The resulting mixture was melted and kneaded in a twin-screw kneader-extruder (PCM-30; made by Ikegai Tekko K. K.) and, after having been cooled, the kneaded mixture was pulverized in a feather mill and thus a magenta master batch A was obtained.

A yellow master batch A was obtained in the same way as in the case of the magenta master batch A, except that C. I. pigment yellow 180 (secondary agglomerate volume-mean particle size, about 2.5  $\mu\text{m}$ ) was used as chromatic coloring material. Similarly, a cyan master batch A was obtained in the same way as in the case of the magenta master batch A, except that C. I. pigment blue 15-3 (secondary agglomerate volume-mean particle size, about 3  $\mu\text{m}$ ) was used as chromatic coloring material.

## Master Batch Preparation Example 2

Magenta master batch B, yellow master batch B, and cyan master batch B were obtained in the same way as in Master Batch Preparation Example 1, except that the period of material mixing was changed to 10 minutes.

## Master Batch Preparation Example 3

Magenta master batch C, yellow master batch C, and cyan master batch C were obtained in the same way as in Master Batch Preparation Example 1, except that the loading of hydrophobic silica was changed to 10 g.

## Master Batch Preparation Example 4

Magenta master batch D, yellow master batch D, and cyan master batch D were obtained in the same way as in Master Batch Preparation Example 1, except that the hydrophobic silica (R972) was changed to hydrophobic silica (H2000; made by Hoechst; BET specific surface area, 140  $\text{m}^2/\text{g}$ , 230 g.

## Master Batch Preparation Example 5

Magenta master batch E, yellow master batch E, and cyan master batch E were obtained in the same way as in Master

## 18

Batch Preparation Example 1, except that the hydrophobic silica (972) was changed to hydrophobic titanium dioxide (T805; made by Aerosil Japan; BET specific surface area, 35  $\text{m}^2/\text{g}$ , 230 g.

5

## Master Batch Preparation Example 6

Magenta master batch F, yellow master batch F, and cyan master batch F were obtained in the same way as in Master Batch Preparation Example 1, except that for the polyester resin and chromatic coloring material, those which had been previously ground and disintegrated in a jet mill were used.

## Master Batch Preparation Example 7

Magenta master batch G, yellow master batch G, and cyan master batch G were obtained in the same way as in Master Batch Preparation Example 1, except that a mixture of hydrophobic silica and chromatic coloring material which had been previously mixed and disintegrated in a surface modifier (Hybridization: made by Nara Kikai Seisakusho K. K.) was used as such.

## Master Batch Preparation Example 8

Magenta master batch H, yellow master batch H, and cyan master batch H were obtained in the same way as in Master Batch Preparation Example 1, except that the hydrophobic silica (R972) was not added.

## Master Batch Preparation Example 9

Magenta master batch I, yellow master batch I, and cyan master batch I were obtained in the same way as in Master Batch Preparation Example 2, except that the hydrophobic silica (R972) was not added.

30

## Master Batch Preparation Example 10

Magenta master batch J, yellow master batch J, and cyan master batch J were obtained in the same way as in Master Batch Preparation Example 6, except that the hydrophobic silica (R972) was not added.

40

## Example 13

Magenta master batch A, 150 g, aforesaid polyester resin, 900 g, a negative charge control agent (E-84; made by Orient Kagaku Kogyo K. K.), 10 g, and carnauba wax (made by Kato Yoko K. K.), 20 g were introduced into a 9-liter Henschel mixer (made by Mitsui Kozan K. K.), and mixing was carried out at a peripheral speed of 40 m/sec. for 5 minutes.

50

The resulting mixture was kneaded in a twin-screw extruder-kneader (PCM-30; made by Ikegai Tekko K. K.), and after having been cooled, the kneaded mixture was primarily crushed in a feather mill, and pulverized in a jet mill. Fine particles thus obtained were then minutely classified by an air classifier. As a result, magenta toner particles having a volume-mean particle size of 8.5  $\mu\text{m}$  were obtained. It is to be noted that the volume-mean particle size value is based on measurements by a Coulter counter (made by Coulter Electronics).

60

Toner particles thus obtained, 1 kg, and hydrophobic silica (H2000; made by Hoechst K.K.), 10 g were introduced into a Henschel mixer, and mixing was carried out at a peripheral speed of 20 m/sec for 2 minutes. Thus, magenta toner 25 was obtained.

Yellow toner 25 was obtained in the same way as in the case of magenta toner 25, except that yellow master batch A

65

was used instead of magenta master batch A. Similarly, cyan toner 25 was obtained in the same way as in the case of magenta toner 25, except that cyan master batch A was used instead of magenta master batch A.

#### Example 14

Magenta toner 26, yellow toner 26, and cyan toner 26 were obtained in the same way as in Example 13, except that (magenta, yellow, cyan) master batch B was used instead of (magenta, yellow, cyan) master batch A.

#### Example 15

Magenta toner 27, yellow toner 27, and cyan toner 27 were obtained in the same way as in Example 13, except that (magenta, yellow, cyan) master batch C was used instead of (magenta, yellow, cyan) master batch A.

#### Example 16

Magenta toner 28, yellow toner 28, and cyan toner 28 were obtained in the same way as in Example 13, except that (magenta, yellow, cyan) master batch D was used instead of (magenta, yellow, cyan) master batch A.

#### Example 17

Magenta toner 29, yellow toner 29, and cyan toner 29 were obtained in the same way as in Example 13, except that (magenta, yellow, cyan) master batch E was used instead of (magenta, yellow, cyan) master batch A.

#### Example 18

Magenta toner 30, yellow toner 30, and cyan toner 30 were obtained in the same way as in Example 13, except that (magenta, yellow, cyan) master batch F was used instead of (magenta, yellow, cyan) master batch A.

#### Example 19

Magenta toner 31, yellow toner 31, and cyan toner 31 were obtained in the same way as in Example 13, except that (magenta, yellow, cyan) master batch G was used instead of (magenta, yellow, cyan) master batch A.

#### Comparative Example 13

Magenta toner 32, yellow toner 32, and cyan toner 32 were obtained in the same way as in Example 13, except that (magenta, yellow, cyan) master batch H was used instead of (magenta, yellow, cyan) master batch A.

#### Comparative Example 14

Magenta toner 33, yellow toner 33, and cyan toner 33 were obtained in the same way as in Example 13, except that (magenta, yellow, cyan) master batch I was used instead of (magenta, yellow, cyan) master batch A.

#### Comparative Example 15

Magenta toner 34, yellow toner 34, and cyan toner 34 were obtained in the same way as in Example 13, except that (magenta, yellow, cyan) master batch J was used instead of (magenta, yellow, cyan) master batch A.

#### Comparative Example 16

Magenta toner 35, yellow toner 35, and cyan toner 35 were obtained in the same way as in Example 13, except that

1 kg of polyester resin, 30 g of chromatic coloring material, 10 g of charge control agent, and 20 g of carnauba wax were used as materials for being mixed together at the material mixing step, and that the period of time of mixing was 5 changed to 10 minutes.

Color toners 25-35 obtained in manner as described above were evaluated in respect of color developing performance and transparency in the same way as in the case of Example 1. The results are shown in Table 3.

TABLE 3

|        | Color toner | Master batch | Metal oxide | Color develop property | Transparency |
|--------|-------------|--------------|-------------|------------------------|--------------|
| Ex. 13 | 25          | A            | Added       | ○                      | ◎            |
| Ex. 14 | 26          | B            | Added       | ○~◎                    | ◎            |
| Ex. 15 | 27          | C            | Added       | ○                      | △~○          |
| Ex. 16 | 28          | D            | Added       | ○                      | ◎            |
| Ex. 17 | 29          | E            | Added       | ○                      | ○            |
| Ex. 18 | 30          | F            | Added       | ○~◎                    | ◎            |
| Ex. 19 | 31          | G            | Added       | ◎                      | ◎            |
| Comp.  | 32          | H            | Not added   | x~○                    | x            |
| Ex. 13 |             |              | added       |                        |              |
| Comp.  | 33          | I            | Not added   | △                      | x~△          |
| Ex. 14 |             |              | added       |                        |              |
| Comp.  | 34          | J            | Not added   | △                      | △            |
| Ex. 15 |             |              | added       |                        |              |
| Comp.  | 35          | —            | Not added   | x                      | x            |
| Ex. 16 |             |              |             |                        |              |

30 In the following examples and comparative examples, polyester resin A pulverized to a volume-mean particle size of about 0.8 mm was used as binder resin.

#### Example 20

35 First, 150 g of hydrophobic silica (H-2000; made by Hoechst Industry; BET specific surface area, 140 m<sup>2</sup>/g), as metal oxide particulate, were introduced into a 9-liter capacity Henschel mixer (made by Mitsui Kozan K. K.), and disintegrated at a peripheral speed of 40 m/sec. for 90 sec. Then, 1 kg of the binder resin, 30 g of chromatic coloring material, C. I. pigment red 81 (secondary agglomerate volume mean particle size, about 2.5 μm), and 30 g of the disintegrated hydrophobic silica were introduced into the 40 Henschel mixer and subjected to first stage mixing at a peripheral speed of 40 m/sec. for 30 minutes. Into the resulting mixture were introduced a negative charge control agent (E-84; made by Orient Kagaku Kogyo K. K.), 5 g, and a carnauba wax (made by Kato Yoko K. K.), 20 g, and 45 second stage mixing was carried out for 5 minutes at a peripheral speed of 40 m/sec. Into the mixture thus obtained 50 were introduced 250 g of collected dust-size toner particles, and third-stage mixing was carried out at a peripheral speed of 40 m/sec. for 10 minutes.

55 The resulting mixture was kneaded in a twin-screw extruder-kneader (PCM-30; made by Ikegai Tekko K. K.) and, after having been cooled, the kneaded mixture was primarily crushed in a feather mill, and then the resulting coarse particles were pulverized in a jet mill. Fine particles 60 thus obtained were minutely classified by means of an air classifier. As a result, magenta toner 36 having a volume-mean particle size of 8.0 μm was obtained.

Yellow toner 36 was obtained in the same way as the magenta toner 36, except that C. I. pigment yellow 180 (secondary agglomerate volume-mean particle size, about 3 μm) was used as chromatic coloring material. Similarly, 65 cyan toner 36 was obtained in the same way as the magenta

## 21

toner 36, except that C. I. pigment blue 15-3 (secondary agglomerate volume-mean particle size, about 2.5  $\mu\text{m}$ ) was used as chromatic coloring material.

## Example 21

Magenta toner 37, yellow toner 37, and cyan toner 37 were obtained in the same way as in Example 20, except that the quantity of addition of the hydrophobic silica was 10 g.

## Example 22

Magenta toner 38, yellow toner 38, and cyan toner 38 were obtained in the same way as in Example 20, except that hydrophobic titanium dioxide (T805; made by Aerosil Japan; BET specific surface area, 35  $\text{m}^2/\text{g}$ ), 30 g, was used instead of hydrophobic silica.

## Example 23

Magenta toner 39, yellow toner 39, and cyan toner 39 were obtained in the same way as in Example 20, except that the hydrophobic silica used was R972 (made by Aerosil Japan; BET specific surface area, 110  $\text{m}^2/\text{g}$ ), 30 g.

## Example 24

Magenta toner 40, yellow toner 40, and cyan toner 40 were obtained in the same way as in Example 20, except that mixing at the first mixing step was carried out for 20 minutes.

## Comparative Example 17

Magenta toner 41, yellow toner 41, and cyan toner 41 were obtained in the same way as in Example 20, except that mixing was carried out in one stage and not in two separate stages (first mixing, second mixing) and that the period of mixing was 40 minutes.

## Comparative Example 18

Magenta toner 42, yellow toner 42, and cyan toner 42 were obtained in the same way as in Example 20, except that there was no loading of hydrophobic silica.

## Comparative Example 19

Magenta toner 43, yellow toner 43, and cyan toner 43 were obtained in the same way as in Example 20, except that the first mixing step was carried out in the following way. That is, 100 g of a master batch composed of binder resin and chromatic coloring material pre-kneaded in a high concentration ratio of 7:3; 930 g of binder resin, and 30 g of chromatic coloring material were introduced into a Henschel mixer, and mixing was carried out at a peripheral speed of 40 m/sec for 4 minutes.

Individual toners obtained as described above were evaluated in respect of surface smoothness and absorbance values expressed by relations (1), (2) and (3). Measurements were made in the following way.

First, 4 cc of toluene and 1 g of sample toner were put in a 10 cc screw tube, and rotary mixing was carried out by a vial rotator at 300 rpm to cause the toner to be dissolved. Then, the resulting solution was allowed to drop on a transparent sheet (OHP sheet) and the solution was uniformly coated on the sheet by using a wire-wrapped bar coater while diametrically adjusting the wire wrap so as to provide a dried coat thickness of 10 to 20  $\mu\text{m}$ , and then the coating was dried. Measurement of the dried coat thickness was made by using an eddy current film thickness measuring

## 22

device (made by Fisher K.K.). The glossiness of the toner film thus obtained was measured by using a gloss meter (GM-060; made by Minolta K. K.). The glossiness was calculated from the relation: (reflected luminous flux from sample/reflected luminous flux from standard glass)  $\times 100$ . Measurement was made under the following conditions: angle of incidence and reflection of measured light was fixed at 60°; and glossiness of the standard glass having a refractive index of 1.567 was taken as 100.

Next, with respect to magenta toner (500–600 nm), yellow toner (380–500 nm), and cyan toner (600–800 nm), maximum absorbance in each respective wave range, and minimum absorbance of each toner in a wave range of 400 to 800 nm were measured by using a self-spectrophotometer (U-3200; made by Hitachi Seisakusho K. K.) and, for each respective toner film, spectroral absorbance was determined on the basis of these measurements and in accordance with the relations (1), (2) and (3). The results are shown in Tables 4 to 6.

Documents with stepwise density variations were prepared for each of magenta, yellow, and cyan, and an image of each document was formed on an OHP sheet by using a full-color copying machine CF900 (made by Minolta K. K.). The image was projected onto a screen, and an image portion on the screen which corresponds to a toner film portion having a film thickness of  $10 \mu\text{m} \pm 0.5 \mu\text{m}$  was visually evaluated. Toner film thickness was measured by an eddy current film thickness measuring device (made by Fisher K.K.). In color development evaluation, where good color reproduction was observed, the toner was rated  $\textcircled{O}$ ; where color reproduction was slightly less favorable, the toner was rated  $\textcircled{O}$ ; where color was somewhat dull, the toner was rated  $\Delta$ ; and where color was dull, the toner was rated  $\textcircled{x}$ . In transparency evaluation, where the image was found clear, the toner was rated  $\textcircled{O}$ ; where the image was found slightly less clear, the toner was rated  $\textcircled{O}$ ; where the image was found somewhat dark, the toner was rated  $\Delta$ ; and where the image was found dark, the toner was rated  $\textcircled{x}$ . The results are shown in Tables 4 to 6.

TABLE 4

|        | Magenta Toner | Gloss | $(A_{MP} - A_{MB})/A_{MB}$ | Color develop Property | Transparency      |
|--------|---------------|-------|----------------------------|------------------------|-------------------|
| Ex. 20 | 36            | 115   | 115                        | $\textcircled{O}$      | $\textcircled{O}$ |
| Ex. 21 | 37            | 108   | 93                         | $\textcircled{O}$      | $\textcircled{O}$ |
| Ex. 22 | 38            | 112   | 91                         | $\textcircled{O}$      | $\textcircled{O}$ |
| Ex. 23 | 39            | 113   | 96                         | $\textcircled{O}$      | $\textcircled{O}$ |
| Ex. 24 | 40            | 108   | 88                         | $\textcircled{O}$      | $\textcircled{O}$ |
| Comp.  | 41            | 105   | 79                         | $\textcircled{O}$      | $\Delta$          |
| Ex. 17 |               |       |                            |                        |                   |
| Comp.  | 42            | 102   | 73                         | $\Delta$               | $\Delta$          |
| Ex. 18 |               |       |                            |                        |                   |
| Comp.  | 43            | 95    | 54                         | $\textcircled{x}$      | $\textcircled{x}$ |
| Ex. 19 |               |       |                            |                        |                   |

TABLE 5

|        | Yellow Toner | Gloss | $(A_{VP} - A_{VB})/A_{VB}$ | Color develop property | Transparency      |
|--------|--------------|-------|----------------------------|------------------------|-------------------|
| Ex. 25 | 36           | 125   | 101                        | $\textcircled{O}$      | $\textcircled{O}$ |
| Ex. 26 | 37           | 115   | 82                         | $\textcircled{O}$      | $\textcircled{O}$ |
| Ex. 27 | 38           | 113   | 80                         | $\textcircled{O}$      | $\textcircled{O}$ |

TABLE 5-continued

| Yellow Toner | Gloss | $(A_{VP} - A_{VB})/A_{VB}$ | Color develop property | Transparency |
|--------------|-------|----------------------------|------------------------|--------------|
| Ex. 28       | 39    | 119                        | 85                     | ◎            |
| Ex. 29       | 40    | 110                        | 78                     | ◎            |
| Comp.        | 41    | 102                        | 70                     | ○            |
| Ex. 20       |       |                            |                        | Δ            |
| Comp.        | 42    | 99                         | 64                     | Δ            |
| Ex. 21       |       |                            |                        | Δ            |
| Comp.        | 43    | 98                         | 54                     | Δ            |
| Ex. 22       |       |                            |                        | Δ            |

TABLE 6

| Cyan toner | Gloss | $(A_{CP} - A_{CB})/A_{CB}$ | Color develop property | Transparency |
|------------|-------|----------------------------|------------------------|--------------|
| Ex. 30     | 36    | 110                        | 61                     | ◎            |
| Ex. 31     | 37    | 105                        | 49                     | ◎            |
| Ex. 32     | 38    | 107                        | 48                     | ◎            |
| Ex. 33     | 39    | 107                        | 51                     | ◎            |
| Ex. 34     | 40    | 105                        | 47                     | ◎            |
| Comp.      | 41    | 100                        | 42                     | ○            |
| Ex. 23     |       |                            |                        | ○            |
| Comp.      | 42    | 98                         | 39                     | Δ            |
| Ex. 24     |       |                            |                        | Δ            |
| Comp.      | 43    | 96                         | 29                     | Δ            |
| Ex. 25     |       |                            |                        | x            |

What is claimed is:

1. A method of producing a color toner which comprises the following steps:
  - a first mixing step for mixing a binder resin, a chromatic coloring material, and metal oxide particulate, wherein the weight ratio of the chromatic coloring material to the metal oxide particulate is 10:1-1:5;
  - a second mixing step for mixing the mixture obtained at the first mixing step and a material other than the materials used in the first mixing step;
  - the step of melting and kneading the mixture obtained at the second mixing step;
  - the step of pulverizing the kneaded mixture after the mixture has been cooled; and
  - the step of classifying the resulting pulverized material.
2. A method of producing a color toner as set forth in claim 1, wherein the other material used for mixing in the second mixing step is at least one of a charge control agent and a wax.
3. A method of producing a color toner as set forth in claim 1, further comprising a third mixing step for mixing toner particles collected at the classifying step into the mixture obtained at the second mixing step.
4. A method of producing a color toner as set forth in claim 1, further comprising the step of premixing the chromatic coloring material and the metal oxide particulate prior to the first mixing step.
5. A method of producing a color toner as set forth in claim 1, wherein the metal oxide particulate has a BET specific surface area of 20 to 300 m<sup>2</sup>/g.
6. A method of producing a color toner as set forth in claim 5, wherein the metal oxide particulate is surface-treated with a hydrophobicizing agent.
7. A method of producing a color toner as set forth in claim 1, wherein a melting viscosity V<sub>2</sub> of the binder resin

at 100° C. is 5×10<sup>4</sup> to 1×10<sup>6</sup> poise, and a ratio V<sub>1</sub>/V<sub>2</sub> of melting viscosity V<sub>1</sub> of the binder resin at 90° C. to the melting viscosity V<sub>2</sub> is 8 or more.

8. A method of producing a color toner which comprises the following steps:

5 a first mixing step for mixing a binder resin having a mean particle size of 1 to 3 mm, and a chromatic coloring material;

a second mixing step for mixing the mixture obtained at the first mixing step and a binder resin having a mean particle size of 0.1 to 0.5 mm;

a step of melting and kneading the mixture obtained at the second mixing step;

a step of pulverizing the kneaded mixture after the mixture is cooled; and

a step of classifying the resulting pulverized material.

9. A method of producing a color toner as set forth in claim 8, further comprising a third mixing step for mixing materials other than those used in the first and second material mixing steps.

10. A method of producing a color toner as set forth in claim 8, wherein at the second mixing step a material other than those used at the first mixing step is mixed along with the binder resin having a mean particle size of 0.1 to 0.5 mm.

11. A master batch for use in a color toner comprising: a binder resin, 20 to 100 parts by weight of a chromatic coloring material relative to 100 parts by weight of the binder resin, and metal oxide particulate.

12. A master batch as set forth in claim 11, wherein the weight ratio of the chromatic coloring material to the metal oxide particulate (coloring material:metal oxide) is 10:1 to 1:5.

13. A master batch as set forth in claim 11, wherein the metal oxide particulate has a BET specific surface area of 20 to 300 m<sup>2</sup>/g.

14. A master batch as set forth in claim 13, wherein the metal oxide particulate is surface-treated with a hydrophobicizing agent.

15. A method of producing a color toner which comprises the following steps:

a master batch preparing step for preparing a master batch containing a binder resin, 20 to 100 parts by weight of a chromatic coloring agent relative to 100 parts by weight of the binder resin, and metal oxide particulate;

a first mixing step for mixing the master batch and a binder resin;

a second mixing step for mixing the mixture obtained at the first mixing step and a material other than the materials used in the first mixing step;

a step of melting and kneading the mixture obtained; a step of pulverizing the kneaded mixture after the mixture is cooled; and

a step of classifying the resulting pulverized material.

16. A method of producing a color toner as set forth in claim 15, wherein the chromatic coloring material content of the color toner is 1 to 10 parts by weight relative to 100 parts by weight of the binder resin.

17. A magenta toner comprising:

at least a binder resin and a magenta pigment; wherein when a film of the magenta toner is formed on a sheet for an overhead projector, the toner film has a surface gloss of 105 or more and satisfies the following relation (1):

$$(A_{MP} - A_{MB})/A_{MB} \geq 85 \quad (1)$$

65 in which A<sub>MP</sub> denotes maximum absorbance of the toner film in a wave range of 500 to 600 nm, and A<sub>MB</sub> denotes minimum absorbance in a wave range of 400 to 800 nm.

**25**

**18.** A magenta toner as set forth in claim **17**, further containing metal oxide particulate having a BET specific surface area of 20 to 300 m<sup>2</sup>/g.

**19.** A magenta toner as set forth in claim **17**, wherein a melting viscosity V<sub>2</sub> of the binder resin at 100° C. is 5×10<sup>4</sup> to 1×10<sup>6</sup> poise, and a ratio V<sub>1</sub>/V<sub>2</sub> of melting viscosity V<sub>1</sub> of the binder resin at 90° C. to the melting viscosity V<sub>2</sub> is 8 or more.

**20.** A yellow toner comprising:

at least a binder resin and a yellow pigment; wherein when a film of the yellow toner is formed on a sheet for an overhead projector, the toner film has a surface gloss of 105 or more and satisfies the following relation (2):

$$(A_{YP}-A_{YB})/A_{YB} \geq 75 \quad (2)$$

in which A<sub>YP</sub> denotes maximum absorbance of the toner film in a wave range of 380 to 500 nm, and A<sub>YB</sub> denotes minimum absorbance in a wave range of 400 to 800 nm.

**21.** A yellow toner as set forth in claim **20**, further containing metal oxide particulate having a BET specific surface area of 20 to 300 m<sup>2</sup>/g.

**22.** A yellow toner as set forth in claim **20**, wherein a melting viscosity V<sub>2</sub> of the binder resin at 100° C. is 5×10<sup>4</sup>

10

15

20

**26**

to 1×10<sup>6</sup> poise, and a ratio V<sub>1</sub>/V<sub>2</sub> of melting viscosity V<sub>1</sub> of the binder resin at 90° C. to the melting viscosity V<sub>2</sub> is 8 or more.

**23.** A cyan toner comprising:

at least a binder resin and a cyan pigment; wherein when a film of the cyan toner is formed on a sheet for an overhead projector, the toner film has a surface gloss of 105 or more and satisfies the following relation (3):

$$(A_{CP}-A_{CB})/A_{CB} \geq 45 \quad (3)$$

in which A<sub>CP</sub> denotes maximum absorbance of the toner film in a wave range of 600 to 800 nm, and A<sub>CB</sub> denotes minimum absorbance in a wave range of 400 to 800 nm.

**24.** A cyan toner as set forth in claim **23**, further containing metal oxide particulate having a BET specific surface area of 20 to 300 m<sup>2</sup>/g.

**25.** A cyan toner as set forth in claim **23**, wherein a melting viscosity V<sub>2</sub> of the binder resin at 100° C. is 5×10<sup>4</sup> to 1×10<sup>6</sup> poise, and a ratio V<sub>1</sub>/V<sub>2</sub> of melting viscosity V<sub>1</sub> of the binder resin at 90° C. to the melting viscosity V<sub>2</sub> is 8 or more.

\* \* \* \* \*